

## UNITED STATES PATENT OFFICE

JOSEPH BEDO, OF CLEVELAND, OHIO, ASSIGNOR TO PERMACHROME PROCESS CORPORATION, OF CLEVELAND, OHIO, A CORPORATION OF OHIO

## ELECTROPLATING BATH

No Drawing.

Application filed July 5, 1928. Serial No. 290,689.

This invention relates to the electrodeposition of metals and it has particular reference to a plating bath or solution for use in connection with the electrodeposition of chromium upon other metals, particularly aluminum.

It is a fact well known to those skilled in the art that the efficiency of an electro-plating process is largely dependent upon the carrying qualities or "throw" of the bath in which the metal to be deposited is carried in the solution.

The present invention is concerned with a bath or solution for use in connection with the electro-plating of chromium upon other metals, the object of the invention being to provide such a bath or solution which is characterized by a quick "throw" and a more even deposition of the metal carried therein, namely, chromium.

The invention further provides a solution or bath which when used in connection with the process disclosed in a copending application filed jointly by Clyde S. Morgan and myself, Serial No. 285,500, filed June 14, 1928, covering a process of plating aluminum, results in a highly efficient and practical process for depositing chromium upon aluminum, an achievement which has long been sought by those skilled in the art.

My improved plating bath or solution includes, as a novel ingredient, a metallic thiosulphate, particularly a thiosulphate of an alkali metal, such as sodium thiosulphate or potassium thiosulphate. With a metallic thiosulphate such as mentioned above, I employ a compound of the metal to be deposited, such for example as chromic acid if the metal is to be chromium. The metallic thiosulphate and the compound of the metal to be deposited are preferably stirred or mixed, after one is added to the other. They may be combined in different proportions but the preferred proportions are approximately fifty parts of the metallic compound, such as chromic acid and one part of metallic thiosulphate such as the sodium thiosulphate or the potassium thiosulphate.

When these ingredients are mixed I find that a considerable heat is evolved for a time

and, therefore, believe that the ingredients are chemically combined, but I am not certain of the exact chemical action taking place in such combination.

I have found that by using the above described solution in connection with the proper voltage and amperage of electric current, such as commonly employed in electrodepositing chromium or the like, the chromium is deposited quickly and evenly on the metal forming the cathode even though the cathode may be formed of aluminum.

I do not desire to be limited to the precise proportions or ingredients set forth above as these may vary without departing from the spirit of the invention or from the scope of the appended claims, and although the invention has particular utility for the deposition of chromium, particularly on aluminum or aluminum alloys, I do not desire to limit myself to the deposition of this metal or to aluminum or aluminum alloys as a base metal, or to the deposition of the plating metal upon the base metal by any particular process, or to the deposition thereon only after it has been first treated or coated.

Having thus described my invention, what I claim is:

1. An electro-plating bath formed by combining a thiosulphate of an alkali metal, and chromic acid.
2. An electro-plating bath prepared by mixing sodium thiosulphate and chromic acid.

In testimony whereof, I hereunto affix my signature.

JOSEPH BEDO.

90

95

100